

# UNITED STATES PATENT OFFICE.

CARLETON ELLIS, OF MONTCLAIR, NEW JERSEY, ASSIGNOR TO ELLIS-FOSTER COMPANY, A CORPORATION OF NEW JERSEY.

## CLOTH-TINTING COMPOSITION AND PROCESS OF TINTING CLOTH.

1,412,014.

Specification of Letters Patent.

Patented Apr. 4, 1922.

No Drawing.

Application filed July 30, 1921. Serial No. 488,684.

To all whom it may concern:

Be it known that I, CARLETON ELLIS, a citizen of the United States, residing at Montclair, in the county of Essex and State 5 of New Jersey, have invented certain new and useful Improvements in Cloth-Tinting Compositions and Processes of Tinting Cloth, of which the following is a specification.

10 This invention relates to a process of treating the lining of automobile tops and relates especially to a method of spraying a tinting composition on such linings and to a composition adapted for such tinting purposes.

15 The invention is concerned especially with the revival or renewal of the linings of automobile tops such as the ordinary touring car top which has an outer fabric of leather or 20 leather substitute and an inner lining of cloth which is usually loosely attached to the outer covering. The inner cloth lining very quickly becomes weather stained and streaked from water and dust and becomes unsightly.

25 While the outer fabric may be treated with leather dressings to restore its appearance, heretofore there has been no satisfactory way of reviving the interior or lining.

According to the present invention, in its 30 preferred form, a solution is made in a hydrocarbon solvent of a dye which is soluble in such solvent but insoluble in water. The oil soluble dyes now on the market and used in varnish stains may be employed for 35 the purpose. They are sold under various names and are readily obtainable. Ordinarily I prefer to use a stain which gives a brown, drab or mahogany tint. It is desirable to have the solution strong enough in 40 dye to adequately cover the water stains of the fabric. It is also desirable to have present a small amount of resin to better hold the dye in place and to serve to slightly brighten the fabric. On the other hand it is 45 undesirable to use a heavy bodied varnish basis or anything of this description because it renders the fabric stiff and also may lead to spontaneous combustion when the top is closed and the lining is folded and 50 pressed together.

For this reason I prefer to use approximately a two per cent solution of a resin as a binder and brightener. However the proportion of resin may be varied from less 55 than 2% to 10% and upwards. Between

2% and 8% satisfactory results are obtained. The resin is calculated on the weight of solvent employed. The resin also serves to some extent as a waterproofing agent so that when cloth so treated is again exposed to 60 rain water stains do not form as readily.

A suitable solvent vehicle is benzol or toluol but preferably varnish painters' naphtha or heavy benzine is used. A mixture of benzine and benzol may be employed.

65 The proportion of the oil-soluble color may be approximately one per cent but may vary more or less according to the intensity of the tint desired.

A suitable composition is made by dissolving 2% of cumaron resin in a solvent composed of 90% of varnish makers' naphtha and 10% of benzol and adding a mixture of one part of oil-soluble orange stain to two parts of oil-soluble oak stain, the proportion of oil-soluble dye in this case is one per cent. This gives a brownish tone with a slightly reddish tint which quite effectively covers the weather stains on the fabric.

70 If such a composition were applied with a brush it would be difficult to make even application but by means of spraying the composition may be applied uniformly. However if a sprayer does not work properly and drops of the composition fall on the fabric the resulting blot is difficult to 75 cover by subsequent coats of the composition as applied by spraying.

75 However I find that it is possible to apply the spray to the cloth from the underside 80 when the cloth is in a horizontal position as for example in its normal position in the automobile top.

One feature of the invention therefore is 85 that of spraying a composition of this character in a substantially vertical position against the fabric thereby overcoming the danger of not securing a uniform application. Hence it is possible to treat the fabric 90 in the automobile top without its removal 95 from the machine.

100 Other resins or binders such as shellac, ordinary rosin, rosin ester and drying oils such as linseed oil, wood oil, etc., may likewise be used in some cases. However a 105 resin which is substantially unaffected by water, that is does not turn white or change in appearance on contact with water is preferred.

110 Other mixtures may be used which have a

water-proofing effect as for example a solution of paraffin or better ceresin wax in benzol or toluol. This is tinted with the oil soluble dye. 2 or 3% of wax suffices to secure desirable waterproofing results but the wax may be increased if desired. Non-inflammable solvents such as trichlorethylene or carbon tetrachloride may be used.

Ordinarily a quick drying composition is desired as the fabric is preferably quite thoroughly wetted with the solution and with slow drying materials present the lining would require a protracted exposure in order to render the fabric perfectly dry. By the use of small quantities of resin in this manner a binding effect may be secured without the employment of drying oil.

Other solutions such as alcoholic solutions of dyestuffs which are insoluble in water may likewise be employed but as a rule do not give as satisfactory results. It is also possible to spray a water soluble dye as for example an aqueous solution of a dyestuff on the fabric and subsequently treat with a mordant or fixative. However the present

process involving the use of a dilute resin solution containing an oil-soluble but water insoluble dyestuff and sprayed vertically against the fabric accomplishes very satisfactory results at a low cost and with a simplicity of operation which is desirable. The top does not have to be removed from the body of the car in order to treat it. This preferred method therefore is recommended for the majority of automobile top linings. 35

What I claim is:—

1. A composition for treating the fabric lining of automobile tops which comprises a dilute solution of a resin carrying oil-soluble dye. 40

2. A composition for treating the fabric lining of automobile tops which comprises a dilute solution of a resin carrying a 2% solution of an oil-soluble and water insoluble dye. 45

3. A composition for treating automobile top linings which comprises a 2% solution of cumaron resin and 1% of oil-soluble but water insoluble dye.

CARLETON ELLIS.